

# United States Patent Office

3,486,897

Patented Dec. 30, 1969

1

3,486,897

**3,486,697**  
**MEROXYANINE DYES AS FILTER DYES AND**  
**SPECTRAL SENSITIZERS**

Gene Leech Oliver, Rochester, N.Y., assignor to Eastman Kodak Company, Rochester, N.Y., a corporation of New Jersey  
No Drawing. Filed July 22, 1966, Ser. No. 567,070  
Int. Cl. G03c 1/84, 1/10

**U.S. Cl. 96—84** **21 Claims**

**U.S. Cl. 96—84** **21 Claims**

21 Claims

## ABSTRACT OF THE DISCLOSURE

Certain merocyanine dyes derived from cyanomethyl sulfones are useful as filter dyes and as spectral sensitizers in light-sensitive photographic silver halide emulsions. 2-(3-cyano-3-dodecylsulfonylallylidene)-3-ethylthiazoline and 2-(3-cyano-3-dodecylsulfonylallylidine)-3-(3-sulfopropyl)thiazolidine, potassium salt are illustrative of the merocyanine dyes.

This invention relates to novel and improved photographic materials, and more particularly to light-sensitive photographic silver halide emulsions containing certain merocyanine dyes derived from cyanomethyl sulfones as filter and sensitizing dyes therein, to novel merocyanine dyes of the above kind, and to the preparation of these materials and dyes.

It is known to employ light-screening substances in photographic elements for antihalation purposes and for protecting a light-sensitive emulsion or emulsions from the action of light which it is not desired to record. For example, light-screening substances are often required (a) in backing layers on either side of the support to reduce halation, (b) in overcoats on photographic elements to protect the light-sensitive emulsion or emulsions from the effects of ultraviolet light, particularly in the case of color photographic elements, and (c) in interlayers between differentially color-sensitized emulsions to protect an underlying emulsion layer or layers from unwanted action of certain wavelengths of light. However, many of the light-screening substances that have been employed for the purposes indicated above are not resistance to diffusion and wander from their desired position or positions in the photographic element. Furthermore, many of them do not have sufficiently sharp absorption maxima and high extinction coefficients in the desired regions of the spectrum.

I have now made the important discovery that certain merocyanine dyes derived from cyanomethyl sulfones are especially useful as filter dyes and sensitizers in light-sensitive photographic silver halide emulsions. These dyes not only have desirably sharp absorption maxima and high extinction coefficients, but also show very high resistance to diffusion and remain firmly fixed in the applied positions in the photographic element. They are further characterized by providing photographic filter layers which absorb to appreciably shorter wavelengths in the ultraviolet region of the spectrum as compared with similar layers prepared with any of the previously known related dimethine type of dyes. This is of particular advantage in certain photographic applications. The dyes are further useful for the preparation of non-light sensitive photographic elements such as diffusion transfer sheets (color and black-and-white), etc.

It is, accordingly, an object of this invention to provide novel and improved photographic materials, and more particularly light-sensitive photographic silver halide emulsions containing at least one of the merocyanine dyes of the invention.

Another object of this invention is to provide novel and

2

improved light-sensitive photographic elements comprising a support material having thereon at least one layer of the above novel emulsions of the invention.

Another object of this invention is to provide novel and improved light-sensitive photographic elements comprising a support material having thereon at least one light sensitive silver halide emulsion layer and at least one light-absorbing filter layer comprising a merocyanine dye of the invention.

10 Another object of this invention is to provide novel  
merocyanine dyes derived from cyanomethyl sulfones  
which absorb in the ultraviolet region of the spectrum,  
which have sharp absorption maxima and high extinction  
coefficients, and which have low diffusibility in the photo-  
15 graphic layers of the invention.

Other objects will become apparent from the following description and examples.

The novel merocyanine dyes which are suitable for accomplishing the above objects of my invention include 20 those represented by the following general formula:



25 where each of  $n$  and  $m$  represents a positive integer of from 1 to 2; R represents a hydrogen atom, an alkyl group (including substituted alkyl) and preferably containing about from 1 to 8 carbon atoms, e.g., methyl, ethyl, propyl, isopropyl, butyl, hexyl, octyl, etc., an aryl group, e.g., phenyl, chlorophenyl, tolyl, etc., or an aralkyl group, e.g., benzyl, phenylethyl, etc.;  $R_1$  represents an alcohol radical, e.g., an alkyl substituent (including substituted alkyl) and preferably containing from 1 to 12 carbon atoms, e.g., methyl, sulfoethyl, carboxyethyl, hydroxypropyl, sulfobutyl, carboxybutyl, hexyl, octyl, dodecyl, etc., or an aryl group, e.g., phenyl, sulfophenyl, carboxyphenyl, tolyl, etc.;  $R_2$  represents an alkyl group (including substituted alkyl) and preferably containing from 1 to 12 carbon atoms, e.g., methyl, ethyl, propyl, isopropyl, butyl, hexyl, octyl, dodecyl, etc., an aryl group, e.g., phenyl, tolyl, naphthyl, etc., an aralkyl group, e.g., benzyl, phenylethyl, etc., or a nitrogen heterocyclic group attached to the sulfonyl group through a nuclear carbon atom such as an oxazolyl group, a benzoxazolyl group, a pyridyl group, a quinolyl group, an imidazolyl group and a benzimidazolyl group, and Z represents the nonmetallic atoms required to complete a 5- to 6- membered heterocyclic nucleus such as those selected from the class consisting of a thiazole nucleus (e.g., thiazole, 4-methylthiazole, 4-phenylthiazole, 5-methylthiazole, 5-phenylthiazole, 4,5-dimethylthiazole, 4,5-diphenylthiazole, 4-(2-thienylthiazole, etc.), a benzothiazole nucleus (e.g., benzothiazole, 4-chlorobenzothiazole, 5-chlorobenzothiazole, 6-chlorobenzothiazole, 7-chlorobenzothiazole, 4-methylbenzothiazole, 5 - methylbenzothiazole, 6 - methylbenzothiazole, 5-bromobenzothiazole, 6-bromobenzothiazole, 4 - phenylbenzothiazole, 5 - phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5 - hydroxybenzothiazole, 6-hydroxybenzothiazole, etc.), a naphthothiazole nucleus, (e.g.,  $\alpha$ -naphthothiazole,  $\beta$ -naphthothiazole, 5-methoxy- $\beta$ ,  $\beta$  - naphthothiazole, 5 - ethoxy -  $\beta$ -naphthothiazole, 8-methoxy -  $\alpha$ -naphthothiazole, 7-methoxy- $\alpha$ -naphthothiazole, etc.), a thionaphtheno-7',6', 4,5-thiazole nucleus (e.g., 4' - methoxythianaphtheno - 7',6',4,5 - thiazole, etc.), an oxazole nucleus (e.g., 4-methyloxazole, 5-methyloxazole, 4-phenyloxazole, 4,5-diphenyloxazole, 4-ethyloxazole, 4,5-dimethyloxazole, 5-phenyloxazole, etc.), a benzoxazole

3

nucleus (e.g., benzoxazole, 5-chlorobenzoxazole, 5-methylbenzoxazole, 5 - phenylbenzoxazole, 6 - methylbenzoxazole, 5,6-dimethylbenzoxazole, 4,6-dimethylbenzoxazole, 5-methoxybenzoxazole, 5-ethoxybenzoxazole, 5-chlorobenzoxazole, 6-methoxybenzoxazole, 5-hydroxybenzoxazole, 6-hydroxybenzoxazole, etc.) a naphthoxazole nucleus (e.g.,  $\alpha$ -naphthoxazole,  $\beta$ -naphthoxazole, etc.), a selenazole nucleus (e.g., 4-methylselenazole, 4-phenylselenazole, etc.), a benzoselenazole nucleus (e.g., benzoselenazole, 5 - chlorobenzoselenazole, 5 - methoxybenzoselenazole, 5-hydroxybenzoselenazole, tetrahydrobenzoselenazole, etc.), a naphthoselenazole nucleus (e.g.,  $\alpha$ -naphthoselenazole,  $\beta$ -naphthoselenazole, etc.), a thiazoline nucleus (e.g., thiazoline, 4-methylthiazoline, etc.), a 2-pyridine nucleus (e.g., 2-pyridine, 2-methyl-2-pyridine, etc.), a 4-pyridine nucleus (e.g., 4-pyridine, 3-methyl-4-pyridine, etc.), a 2-quinoline nucleus (e.g., 2-quinoline, 3 - methyl - 2-quinoline, 5-ethyl-2-quinoline, 6-chloro-2-quinoline, 8-chloro-2-quinoline, 6-methoxy-2-quinoline, 8-ethoxy-2-quinoline, 8-hydroxy-2-quinoline, etc.), a 4-quinoline nucleus (e.g., 4-quinoline, 6-methoxy-4-quinoline, 7-methyl-4-quinoline, 8-chloro-4-quinoline, etc.), a 1-isoquinoline nucleus (e.g., 1-isoquinoline, 3,4-dihydro-1-isoquinoline, etc.), a 3-isoquinoline nucleus (e.g., 3-isoquinoline, etc.), a 3,3-dialkylinolenine nucleus, an imidazole nucleus (e.g., imidazole, 1-alkylimidazole, 1-alkyl - 4-phenylimidazole, 1-alkyl-4,5-dimethylimidazole, etc.), a benzimidazole nucleus (e.g., benzimidazole, 1-alkylenzimidazole, 1 - aryl - 5,6-dichlorobenzimidazole, etc.), a naphthimidazole nucleus (e.g., 1-alkyl- $\alpha$ -naphthimidazole, 1-aryl- $\beta$ -naphthimidazole, 1-alkyl-5-methoxy- $\alpha$ -naphthimidazole, etc.), etc.

The above defined merocyanine dyes of the invention can conveniently be prepared, for example, by condensing a cyanomethyl sulfone corresponding to the formula  $R_2-SO_2-CH_2-CN$ , wherein  $R_2$  is as previously defined, (prepared, for example, by the general method of Dijkstra and Backer, Rec. Trav. Chim., 73, 569 (1954)) with (1) derivatives of heterocyclic bases such as those represented by the general formula:



wherein  $m$ ,  $n$ ,  $R_1$  and  $Z$  are as previously defined,  $R_3$  represents an acyl group, e.g., acetyl, propionyl, benzoyl, etc.,  $R_4$  represents an aryl group, e.g., phenyl or tolyl, and  $X$  represents an acid anion, e.g., chloride, bromide, iodide, *p*-toluenesulfonate, sulfamate, methyl sulfate, ethyl sulfate, perchlorate, etc., or (2) compounds represented by the general formula:



wherein  $n$ , R, R<sub>1</sub>, X and Z are as previously defined, and R<sub>5</sub> represents methyl or ethyl, in an inert solvent medium e.g., alkanol such as methanol, butanol, etc., acetone, 1,4-dioxane, pyridine, dimethylformamide, dimethylacetamide, quinoline, and the like, at elevated temperatures and preferably at refluxing temperatures of the reaction mixture, in the presence of a basic condensing agent such as a trialkylamine, e.g., triethylamine, tri-n-propylamine, tri-n-butylamine, etc., N-methylpiperidine, N-ethylpiperidine, N,N-dimethylaniline, etc. The dye compounds are then separated from the reaction mixtures by chilling and dilution with nonsolvents such as water, alkanols such as methanol, ethanol, etc. and purified by one or more recrystallizations from suitable solvents such as above and mixtures of solvents, for example, pyridine and methanol.

The intermediate heterocyclic compounds represented

4

by Formulas II and III above are all well known substances, and methods for preparing these compounds are well known to the art. For example, many of them are described in Brooker et al., U.S. Reissue Patent No. 24,292, issued Mar. 19, 1957, and Heseltine et al., U.S. Patent No. 3,140,182, issued July 7, 1964.

The following examples further illustrate this invention.

### EXAMPLE 1

2 - (3 - cyano - 3-methylsulfonylallylidene)-3-ethylbenzothiazoline



A mixture of 2 -  $\beta$  - acetanilidovinyl-3-ethylbenzothiazolium iodide (3.15 g., 7 mmole), methylsulfonylacetone-tri (0.83 g., 7 mmole) and pyridine (10 ml.) was warmed almost to the solution point and triethylamine (1.5 ml., 10.5 mmole) was then added. The resulting mixture was refluxed gently for 5 minutes, cooled and treated with ice and water to precipitate the dye as an oil which after solidification was collected on a filter and dried (1.62 g., 76%). Recrystallization twice from pyridine and methanol afforded the pure dye, M.P. 218-219° C., in 63% yield.

### EXAMPLE 2

## 2 - (3 - cyano - 3-dodecylsulfonylallylidene)-3-ethylbenzoxazoline



A mixture of 2 -  $\beta$  - acetanilidovinyl - 3 - ethylbenzoxazolium iodide (4.34 g., 10 mmole), dodecylsulfonylacetone (2.73 g., 10 mmole), acetic anhydride (0.9 ml.), pyridine (15 ml.) and triethylamine (2.8 mg., 20 mmole) was boiled under reflux for 5 minutes, cooled and diluted with water. The aqueous suspension of oil was extracted twice with ether, the extracts were combined and the ether was removed by evaporation. The residue was taken up in a minimum of warm ethanol, the solution was cooled and the crystalline product collected (2.48 g., 52%). Recrystallization twice from methanol afforded the pure dye M.P. 84-84.5° C. in 39% yield.

**EXAMPLE 3**

2 - (3 - cyano - 3-dodecylsulfonylallylidene)-3-ethyl-thiazolidine



2 -  $\beta$  - anilinovinyl - 3-ethyl-2-thiazolinium iodide (3.62 g., 10 mmole), dodecylsulfonylacetone (2.73 g., 10 mmole), pyridine (15 ml), acetic anhydride (1.9 ml., 20 mmole), and triethylamine (2.8 ml., 20 mmole) were refluxed for 8 minutes and then cooled. The crystals which separated on addition of ice and water were collected on a filter, washed with methanol, and dried (3.52 g., 86%). Recrystallization twice from methanol afforded a 58% yield of the pure dye, M.P. 113-115° C.

**5**  
**EXAMPLE 4**

2 - (3 - cyano - 2-methyl-3-methylsulfonylallylidene)-3-ethylbenzothiazoline



3 - ethyl - 2 - thioacetylidynebenzothiazoline (3.52 g., 15 mmole) and methyl-p-toluenesulfonate (2.79 g., 15 mmole) were heated on a steam bath with dimethylacetamide (5 ml.) for 10 minutes, whereupon the melt solidified. The resulting mixture was diluted with dimethylacetamide (10 ml.), methylsulfonylacetone (1.79 g., 15 mmole) was added, and the mixture was heated on a steam bath to dissolve the reactants. Triethylamine (3.2 ml., 22.5 mmole) was then added and heating was continued for 10 minutes. The mixture was then rapidly brought to a boil to expel methyl mercaptan and allowed to cool. Dilution with ice and water precipitated an oil which crystallized on cooling (3.31 g., 69%). Recrystallization twice from pyridine and methanol afforded the pure dye, M.P. 226-227° C., in 26% yield.

**EXAMPLE 5**

2 - (3 - cyano - 2-methyl-3-methylsulfonylallylidene)-3-ethyl-naphtho[1,2-d]thiazoline



This dye was prepared from 1-ethyl-2-thioacetylidyne-naphtho[1,2-d]thiazoline and methylsulfonylacetone by the method of Example 4. The pure dye, M.P. 252-253° C. from pyridine and methanol, was obtained in 25% yield.

**EXAMPLE 6**

2-(5-cyano-5-methylsulfonyl-2,4-pentadienylidene)-3-ethylbenzothiazoline



2 - (4 - acetanilido - 1,3 - butadienyl) - 3 - ethylbenzothiazonium iodide (2.38 g., 5 mmole), methylsulfonylacetone (1.19 g., 10 mmole), 1,4-diazabicyclo[2.2.2]octane (1.12 g., 10 mmole) and dimethylacetamide (10 ml.) were refluxed for 4 minutes. The resulting mixture was allowed to cool and was then diluted with methanol (30 ml.), chilled, and filtered. The crude dye obtained (1.14 g., 69%) was recrystallized twice from pyridine-methanol to obtain the pure dye, M.P. 205-206° C., in 56% yield.

**EXAMPLE 7**

2-(3-cyano-3-methylsulfonylallylidene)-1-ethyl-naphtho[1,2-d]thiazoline



**6**

A mixture of 2-anilinovinyl-1-ethylnaphtho[1,2-d]thiazolium iodide (3.52 g. 7 mmole), methylsulfonylacetone (0.84 g., 7 mmole), acetic anhydride (1.32 ml., 14 mmole) and dimethylacetamide (15 ml.) was heated; triethylamine (1.96 ml., 14 mmole) was added; and the mixture was refluxed for 2 minutes. The resulting solution was cooled, diluted with 40 ml. of methanol, chilled, and the crude dye collected on a filter (2.45 g., 98%). Recrystallization of the crude dye from pyridine and methanol afforded the pure dye, M.P. 268-269° C., in 67% yield.

**EXAMPLE 8**

2-(3-cyano-3-dodecylsulfonylallylidene)-1-ethyl-naphtho[1,2-d]thiazoline



This dye was prepared from 2-anilinovinyl-1-ethylnaphtho[1,2-d]thiazolium iodide and dodecylsulfonylacetone by the method of Example 7. The pure dye, M.P. 155-156° C. from methanol, was obtained in 69% yield.

**EXAMPLE 9**

2-(3-cyano-3-dodecylsulfonylallylidene)-3-(3-sulfo-propyl)thiazolidine, potassium salt



Anhydro - 2 - anilinovinyl - 3 - sulfopropyl - 2 - thiazolidinium hydroxide (3.26 g., 10 mmole), dodecylsulfonylacetone (2.73 g., 10 mmole), acetic anhydride (1.9 ml., 20 mmole), dimethylacetamide (15 ml.) and triethylamine (2.8 ml., 20 mmole) were heated slowly from 100 to 170° C. over about 5 minutes to obtain a clear, dark solution. The solution was cooled and diluted with ether to precipitate the crude dye which was washed several times with ether. The crude dye was dissolved in ethanol and treated with an ethanolic solution of potassium acetate (1.07 g., 11 mmole) to precipitate the potassium salt of the dye. The resulting suspension was heated to boiling, treated with ethanol until solution was almost complete, and chilled. The crude product (3.48 g., 64%) was then collected on a filter and recrystallized twice from ethanol containing 15-20% water to obtain the pure dye salt, M.P. 218-220° C., in 39% yield.

**EXAMPLE 10**

2-(3-cyano-3-dodecylsulfonylallylidene)-3-(3-sulfo-propyl)benzoxazoline, sodium salt



This dye was prepared by a procedure similar to that employed in Example 9. The pure dye salt, M.P. 251-253° C., was obtained in 41% yield.

7  
EXAMPLE 11

2-(3-o-carboxyphenylsulfonyl-3-cyanoallylidene)-1-ethyl naphtho[1,2-d]thiazoline



2-anilinovinyl-1-ethylnaphtho[1,2-d]thiazolium iodide (3.52 g., 7 mmol.), o-carboxyphenylsulfonylacetone (2.26 g. 10.5 mmol.), acetic anhydride (1.32 ml., 14 mmol.), triethylamine (3.4 ml., 24 mmole.) and dimethylacetamide (10 ml.) were refluxed for two minutes and chilled. Ice, dilute hydrochloric acid, and water were added giving a gum which crystallized on boiling with methanol. The methanol solution was chilled and filtered. The dried precipitate weighed 2.30 g., a 71% yield. On recrystallization from mixtures of dimethylacetamide and acetic acid and dimethylacetamide and methanol, the pure dye, M.P. 234-235° C., was obtained in 49% yield.

## EXAMPLE 12

2-(3-o-carboxyphenylsulfonyl-3-cyano-2-methylallylidene)-1-ethylnaphtho[1,2-d]thiazoline



3-ethyl-2-thioacetonylidenebenzothiazoline (7.13 g., 25 mmol.) and methyl p-toluenesulfonate (5.12 g., 27.5 mmol.) were heated with dimethylacetamide (15 ml.) on the steam bath until the mixture solidified. Then o-carboxyphenylsulfonyl-acetonitrile (30 mmol.), triethylamine (8.7 ml., 60 mmol.) and pyridine (30 ml.) were added and the mixture refluxed for five minutes. The addition of ice and water gave a gummy solid which was taken up in methanol acidified with conc. hydrochloric acid. The dye crystallized when this mixture was boiled and subsequently cooled. The yield was 3.91 g., 33%. It was twice recrystallized from dimethylacetamide from which the dye was thrown out with methanol. The yield of pure dye, M.P. 236-237° C., was 13%.

Among the especially preferred dyes of this invention are those corresponding to above Formula I wherein  $n=1$ ,  $R_1$  represents an alkyl group of from 1-4 carbon atoms bearing a substituent such as a carboxylic acid or sulfonic acid salt group which confers water solubility on the dye, and  $R_2$  represents a group having a molecular weight sufficiently high to prevent a diffusion of the dye in the photographic element. The dye of above Example 9 is particularly efficacious and is preferred.

The dyes of this invention have light-absorbing characteristics that make them valuable for use in light-absorbing filter layers in photographic elements. These characteristics are illustrated in the following Table 1 and in Example 13.

TABLE 1.-ABSORPTION IN METHANOL

| Dye of Example | Maximum (m $\mu$ ) | Coefficient of Extinction $\times 10^{-4}$ |
|----------------|--------------------|--------------------------------------------|
| 1              | 433                | 7.9                                        |
| 2              | 398                | 9.0                                        |
| 3              | 381                | 6.1                                        |
| 4              | 432                | 9.3                                        |
| 5              | 451                | 9.3                                        |
| 6              | 526                | 13.1                                       |
| 7              | 453                | 7.9                                        |
| 8              | 455                | 7.8                                        |
| 9              | 382                | 6.2                                        |
| 10             | 398                | 7.2                                        |
| 11             | 460                | 8.4                                        |
| 12             | 459                | 7.8                                        |

8  
EXAMPLE 13

A composition comprising gelatin, coating aids, hardeners, and the ultraviolet light-absorbing dye of Example 9, 2-(3-cyano-3-dodecylsulfonylallylidene)-3-(3-sulfopropyl)thiazoline, potassium salt, was coated above the blue sensitive layer of a multilayer reversal color film of the type described in Mannes et al. U.S. Patent No. 2,252,718, issued Aug. 19, 1941. The resultant element (a) had 90 mg./ft.<sup>2</sup> of gelatin and 30 mg./ft.<sup>2</sup> of the above dye in the overcoat. A similar element without the light-absorbing overcoat was used as a control. Testing of these coatings by the method recited in U.S. Patent 2,252,718, cited above, gave the following representative sensitometric results:

| Element | Maximum density<br>(fresh test) |       |      | Maximum density change<br>on incubation* |       |       |
|---------|---------------------------------|-------|------|------------------------------------------|-------|-------|
|         | Red                             | Green | Blue | Red                                      | Green | Blue  |
| Control | 3.78                            | 3.42  | 3.78 | 0                                        | 0     | -0.10 |
| A       | 3.78                            | 3.40  | 3.86 | 0                                        | -0.08 | -0.10 |

\* 7 days at 120° F./50% relative humidity, relative to the corresponding fresh coating.

Other sensitometric tests of properties such as minimum density; speed, and metol-hydroquinone developer fog gave results which showed similar agreement between fresh and incubated coatings.

Spectrophotometric exposures demonstrated a significant decrease in ultraviolet sensitivity of the overcoated element A relative to the control element. Practical picture tests confirmed this protection. Pictures obtained with element A gave a color balance similar to those obtained with the control element when the control element was exposed through a Kodak 2A Wratten filter.

Various tests of physical properties which are customarily made on coatings of this type such as vertical swell, fold, wedge brittleness, ferrotyping, gate friction, and the like gave results which indicated that the control element and the overcoated element had essentially equal physical properties.

In the preparation of filter layers for photographic elements such as that illustrated in above Example 13; filter layers between differentially sensitized emulsion layers; filter layers on diffusion transfer receiving sheets such as those described in Land U.S. Patent 2,543,181, issued Feb. 27, 1951; filter layers in or upon color print materials such as those described in Van Campen U.S. Patent 2,956,879, issued Oct. 18, 1960; filter layers in or upon color transfer materials such as those described in British Patent 890,861, dated Mar. 7, 1962, Belgian Patent 636,371, and Rogers U.S. Patents 3,087,817, issued Apr. 30, 1963 and 2,983,606, issued May 9, 1961; and the like; the dyes of this invention are preferably incorporated in colloid layers which are permeable to aqueous processing solutions, said dyes being employed in concentrations which may vary considerably depending upon the particular product concerned and the effect desired. Methods for selecting the particular colloid to be employed, and for determining the amount of dye to be included, are well known in the art and need not be enumerated here. Representative colloids which may be employed include natural materials such as gelatin, protein derivatives, albumin, agar-agar, gum arabic, alginic acid and the like; and synthetic resins such as polyvinyl alcohol, polyvinyl pyrrolidone, polyacrylamide, cellulose ethers and carboxylated derivatives of cellulose ethers, partially hydrolyzed cellulose esters, copolymers of acrylic and methacrylic acids, polymeric latexes or hydrosols, mixtures of these, and the like. Gelatin is the preferred colloid.

In the preparation of photographic silver halide emulsions comprising one or more of the above mentioned colloids, the new dyes of this invention are advantageously incorporated in the washed, finished, silver halide emulsion and should be uniformly distributed throughout the

emulsion. Methods of incorporating dyes in emulsions are relatively simple and well known to those familiar with the art of emulsion making. For example, the dyes may be added from solutions in appropriate solvents which are free from deleterious effects on the ultimate light-sensitive materials. Methanol, isopropanol, and pyridine, alone or in admixture, have proven satisfactory as solvents for incorporating the majority of the dyes of this invention into emulsions.

The types of silver halide emulsions that can be sensitized with the new dyes of this invention include any of the conventional emulsions prepared with light-sensitive silver salts including silver chloride, silver bromide, silver iodide, silver chlorobromide, silver bromoiodide, silver chlorobromo-iodide, etc. The concentration of the new dyes in the emulsion can vary widely, e.g., from about 5 to about 100 mg. per liter of flowable emulsion. The specific concentration will vary according to the type of light-sensitive material in the emulsion and the effects desired. The suitable and most economical concentration for a given emulsion will be apparent to those skilled in the art upon making the tests and observations customarily used in the art of emulsion making.

To prepare a gelatin-silver halide emulsion sensitized with one of the dyes of this invention, the following procedure is satisfactory. A quantity of the dye is dissolved in a suitable solvent and a volume of this solution containing from 5 to 100 mg. of dye is slowly added to about one liter of a gelatin-silver halide emulsion. With most of the dyes, 10 to 20 mg. of dye per liter of emulsion suffices to produce the maximum sensitizing effect with the ordinary gelatin-silver bromide (including bromoiodide and chlorobromide) emulsions. With fine grain emulsions, which include most of the ordinarily employed gelatin-silver chloride emulsions, somewhat larger concentrations of dye may be necessary to obtain the optimum sensitizing effect. While this procedure has dealt with emulsions comprising gelatin, it will be understood that these remarks apply generally to any emulsion wherein part or all of the gelatin is substituted by another suitable hydrophilic colloid, such as previously mentioned. It will also be understood that the above description is intended to be illustrative and should not be construed as limiting my invention in any sense since it is apparent that the new dyes can be incorporated by other methods in many of the photographic silver halide emulsions and hydrophilic colloid layers customarily employed in the art. For instance, the dyes can be incorporated by bathing a plate or film bearing an emulsion layer in a solution of one of the dyes in an appropriate solvent. Bathing methods, however, are not normally preferred.

The following example illustrates photographic elements prepared with the novel silver halide emulsions of the invention.

#### EXAMPLE 14

The sensitizing effects in photographic elements of the new dyes of the invention were determined as follows:

The dyes dissolved in suitable solvents, were added to separate portions of either a silver chloride emulsion or a silver chlorobromide (60:40) emulsion as indicated in Table 2 below, and at the indicated concentrations. After digestion at 50° C. for 10 minutes, the emulsions in each case were coated at a coverage of 432 mg. of silver per square foot and 1190 mg. of gelatin per square foot on a cellulose acetate film support. A sample of each coating was exposed on an Eastman 1B sensitometer and to a wedge spectrograph, processed in a developer of the composition:

G.

|                                |      |
|--------------------------------|------|
| N-methyl-p-aminophenol sulfate | 2.0  |
| Sodium sulfite (anhydrous)     | 90.0 |
| Hydroquinone                   | 8.0  |
| Sodium carbonate (monohydrate) | 52.5 |
| Potassium bromide              | 5.0  |
| Water to make 1.0 liter.       |      |

and then fixed, washed, and dried. The sensitizing results are shown in the following table.

TABLE 2.—SENSITIZING DATA

| Dye of Ex. | Emulsion type   | Dye concentration<br>grams/mole<br>silver | Sensitizing<br>range (m $\mu$ )<br>to — | Sensitizing<br>maximum<br>(m $\mu$ ) |
|------------|-----------------|-------------------------------------------|-----------------------------------------|--------------------------------------|
| 1.         | Chloride        | 0.13                                      | 490                                     | 455                                  |
| 2.         | do              | 0.13                                      | 490                                     | 430                                  |
| 4.         | do              | 0.13                                      | 490                                     | 450                                  |
| 5.         | do              | 0.13                                      | 530                                     | 470                                  |
| 5.         | Chloridebromide | 0.16                                      | 510                                     | 470                                  |
| 6.         | Chloride        | 0.13                                      | 640                                     | 560                                  |
| 6.         | Chloridebromide | 0.08                                      | 640                                     | 550                                  |
| 7.         | do              | 0.13                                      | 530                                     | 480                                  |
| 7.         | Chlorobromide   | 0.16                                      | 530                                     | 470                                  |
| 10.        | Chloride        | 0.13                                      | 450                                     | 410                                  |
| 11.        | Chlorobromide   | 0.13                                      | 530                                     | 485                                  |
| 12.        | do              | 0.13                                      | 525                                     | 470                                  |

Photographic silver halide emulsions containing the sensitizing dyes of this invention can also contain other addenda such as chemical sensitizers, e.g., sulfur sensitizers (e.g., allyl thiocarbamide, thiourea, allylisothiocyanate, cystine, etc.), selenium and tellurium sensitizers, various gold compounds (e.g., potassium chloroaurate, auric trichloride, etc.) (see U.S. Patents to W. D. Baldsiefen, No. 2,540,085, issued Feb. 6, 1951; R. E. Damschroder, No. 2,597,856, issued May 27, 1952; and H. C. Yutzy et al., U.S. Patent No. 2,597,915, issued May 27, 1952), various palladium compounds, such as palladium chloride (W. D. Baldsiefen, U.S. Patent No. 2,540,086, issued Feb. 6, 1951), potassium chloropalladate (R. E. Stauffer et al., U.S. Patent No. 2,598,079, issued May 27, 1952), etc., or mixtures of such sensitizers; antifoggants such as ammonium chloroplatinate (A. P. H. Trivelli et al., U.S. Patent No. 2,566,263, issued Aug. 28, 1951); benzotriazole, nitrobenzimidazole, 5-nitroindazole, benzidine, mercaptans, etc. (see Mees, "The Theory of the Photographic Process," MacMillan Pub., revised edition 1954, page 677), or mixtures thereof.

Photographic silver halide emulsion layers and other layers present in the photographic elements made according to the invention may contain developing agents such as hydroquinones, catchols, 1,3-pyrazolidones, amino-phenols, etc.; and the layers can be hardened with any suitable hardeners such as aldehyde hardeners, aziridine hardeners, hardeners which are derivatives of dioxane, oxy polysaccharides such as oxy starch and oxy plant gums, mixtures of these, and the like. The layers present in photographic elements made according to the invention may also contain color couplers such as those described in I. F. Salminen et al. U.S. Patent No. 2,423,730, issued July 8, 1947; Spence and Carroll U.S. Patent No. 2,640,776, issued June 2, 1953, etc; or mixtures of such addenda. Dispersing agents for color couplers, such as those set forth in U.S. Patents to E. E. Jelley et al. U.S. Patent No. 2,322,027, issued June 15, 1943, and L. D. Mannes et al. U.S. Patent No. 2,304,940, issued Dec. 15, 1942; and non-ionic, anionic and amphoteric coating aids; can also be employed in the above described emulsions and colloid layers. The photographic emulsions can also contain additional additives, particularly those known to be beneficial in photographic emulsion, including, for example, stabilizers, particularly the water soluble inorganic acid salts of cadmium, cobalt, manganese, and zinc, such as disclosed in Jones U.S. Patent No. 2,839,405, issued June 17, 1958, and the substituted triazaindolizines such as disclosed in Heimbach et al. U.S. Patent No. 2,444,605, issued July 6, 1948 and in Heimbach, U.S. Patent No. 2,444,607; spectral sensitizers such as the cyanine, merocyanine, styryl, and hemicyanine dyes; speed increasing materials, such as polyalkylene glycols, onium salts, thioethers, etc.; plasticizers; absorbing dyes; mixtures of these additives; and the like.

Although the photographic element examples show coatings made on cellulose acetate supports, it will be understood that the photographic silver halide emulsions

may be coated advantageously on any of the support materials commonly used in photographic elements, including glass, metals, paper, baryta coated paper, cellulose acetate, cellulose acetate butyrate, cellulose nitrates, etc., and synthetic film forming resinous materials such as polystyrenes, polyolefins, e.g., polyethylene, polypropylene, etc.; such as polyethylene terephthalate, polyamides, e.g., nylon, etc., polycarbonates, polyvinyl acetals, etc. Supports such as papers which are partially acetylated or coated with an  $\alpha$ -olefin polymer, particularly a polymer derived from an  $\alpha$ -olefin containing 2-10 carbon atoms as exemplified by polyethylene and polypropylene, ethylene-butene copolymers, and the like, also give good results.

The invention has been described in detail with particular reference to preferred embodiments thereof, but it will be understood that variations and modifications can be effected within the spirit and scope of the invention as described hereinabove and as defined in the appended claims.

I claim:

1. A light-sensitive photographic silver halide emulsion containing at least one dye compound having the general formula:



wherein  $n$  and  $m$  each represents a positive integer of from 1 to 2,  $R$  represents a member selected from the group consisting of a hydrogen atom, an alkyl group, a monocyclic aryl group and an aralkyl group,  $R_1$  represents a member selected from the group consisting of an alcohol radical and an aryl group,  $R_2$  represents a member selected from the group consisting of an alkyl group, an aryl group, an aralkyl group, an oxazolyl group, a benzoxazolyl group, a pyridyl group, a quinolyl group, an imidazolyl group and a benzimidazolyl group, and  $Z$  represents the nonmetallic atoms required to complete a 5- to 6-membered heterocyclic nucleus selected from the class consisting of a thiazole nucleus, a benzothiazole nucleus, a naphthothiazole nucleus, a thianaphtheno-7',6',4,5-thiazole nucleus, an oxazole nucleus, a benzoxazole nucleus, a naphthoxazole nucleus, a selenazole nucleus, a benzoselenazole nucleus, a naphthoselenazole nucleus, a thiazoline nucleus, a 2-pyridine nucleus, a 4-pyridine nucleus, a 2-quinoline nucleus, a 4-quinoline nucleus, a 1-isoquinoline nucleus, a 3-isoquinoline nucleus, a 3,3-dialkylindolene nucleus, an imidazole nucleus, a benzimidazole nucleus, and a naphthimidazole nucleus.

2. A light-sensitive photographic silver halide emulsion in accordance with claim 1 containing at least one dye compound having the general formula set forth in claim 1 wherein  $R_2$  represents an alkyl group having 1 to 12 carbon atoms.

3. A light-sensitive photographic silver halide emulsion in accordance with claim 1 containing the dye compound 2-(3-cyano-3-dodecylsulfonylallylidene)-3-ethylthiazoline.

4. A light-sensitive photographic silver halide emulsion in accordance with claim 1 containing the dye compound 2-(3-cyano-3-methylsulfonylallylidene)-1-ethylnaphtho-[1,2-d]thiazoline.

5. A light-sensitive photographic silver halide emulsion in accordance with claim 1 containing the dye compound 2-(3-cyano-3-dodecylsulfonylallylidene)-1-ethyl-naphtho-[1,2-d]thiazoline.

6. A light-sensitive photographic silver halide emulsion in accordance with claim 1 containing a water soluble

salt of the dye compound 2-(3-cyano-3-dodecylsulfonylallylidene)-3-(3-sulfopropyl)thiazolidine.

7. A light-sensitive photographic silver halide emulsion in accordance with claim 1 containing the dye compound 2-(3-cyano-3-dodecylsulfonylallylidene)-3-(3-sulfopropyl)thiazolidine, potassium salt.

8. A light-sensitive photographic silver halide emulsion in accordance with claim 1 containing a water soluble salt of the dye compound 2-(3-cyano-3-dodecylsulfonylallylidene)-3-(3-sulfopropyl)benzoxazoline.

9. A light-sensitive photographic silver halide emulsion in accordance with claim 1 containing the dye compound 2-(3-cyano-3-dodecylsulfonylallylidene)-3-(3-sulfopropyl)benzoxazoline, sodium salt.

10. A photographic element comprising a support having thereon at least one silver halide emulsion layer, and wherein at least one of said layers contains a dye compound having the formula set forth in claim 1.

11. A photographic element comprising a support having thereon at least one silver halide emulsion layer, and wherein at least one of said layers contains a dye compound having the formula set forth in claim 2.

12. A photographic element comprising a support having thereon at least one silver halide emulsion layer, and wherein at least one of said layers contains a dye compound defined in claim 6.

13. A photographic element comprising a support having thereon at least one silver halide emulsion layer, and wherein at least one of said layers contains the dye compound defined in claim 7.

14. A photographic element comprising a support, having thereon at least one nonsensitive layer containing a dye compound having the formula set forth in claim 1.

15. A photographic element comprising a support having thereon at least one nonsensitive layer containing a dye compound having the formula set forth in claim 2.

16. A photographic element comprising a support having thereon at least one nonsensitive layer containing a dye compound defined in claim 6.

17. A photographic element comprising a support having thereon at least one nonsensitive layer containing the dye compound defined in claim 7.

18. A photographic element comprising a support having thereon at least one silver halide emulsion layer, and wherein at least one of said layers contains a dye compound having the general formula set forth in claim 1 wherein  $R_2$  represents an aryl group.

19. A photographic element comprising a support having thereon at least one nonsensitive layer containing a dye compound having the formula set forth in claim 1 and having at least one silver halide emulsion layer.

20. A photographic element in accordance with claim 19 wherein a nonsensitive layer is the top layer.

21. A photographic element in accordance with claim 20 wherein a water soluble salt of the dye compound 2-(3-cyano-3-dodecylsulfonylallylidene)-3-(3-sulfopropyl)thiazolidine is present in said nonsensitive top layer.

#### References Cited

#### UNITED STATES PATENTS

|           |         |                |       |        |
|-----------|---------|----------------|-------|--------|
| 2,638,473 | 5/1953  | Edwards        | ----- | 96-102 |
| 2,748,114 | 5/1956  | Brooker et al. | ----- | 96-102 |
| 2,860,984 | 11/1958 | Jones          | ----- | 96-102 |

NORMAN G. TORCHIN, Primary Examiner

M. F. KELLEY, Assistant Examiner

U.S. Cl. X.R.